

# UNITED STATES PATENT OFFICE.

ROBERT R. ROBERTS, OF WASHINGTON, DISTRICT OF COLUMBIA, ASSIGNOR, BY MESNE ASSIGNMENTS, TO WILLIAM J. ROBINSON, OF NEW YORK, N. Y.

## PROCESS OF TREATING FIBROUS MATERIAL.

953,010.

Specification of Letters Patent. Patented Mar. 22, 1910.

No Drawing.

Application filed May 26, 1909. Serial No. 498,576.

*To all whom it may concern:*

Be it known that I, ROBERT R. ROBERTS, a citizen of the United States, residing at Washington, in the District of Columbia, 5 have invented certain new and useful Improvements in Processes of Treating Fibrous Material, of which the following is a description.

My invention relates to the separation of 10 fibers from the stalks of fiber bearing plants such as flax, ramie, jute, hemp, pita and other plants which contain fibers capable for use for the manufacture of textile fabrics, cordage or paper and consists in the process 15 hereinafter described and particularly pointed out in the claims.

The stalks of fiber bearing plants are composed in addition to the fibers, of woody material containing little or no fiber or at 20 least none of commercial value but containing resinous or gummy substances and closely associated with the fiber. It is of course necessary to separate the fiber from this woody portion of the stalk in order to 25 make use of the fiber and this separation of the fiber and woody material has been effected heretofore only with great difficulty and expense. For instance in order to obtain from flax the fiber contained in it the 30 only commercially practicable process has been that of slow rotting or "retting" of the woody material under or in the presence of water. This process is expensive because of the length of time and the care and attention required and also because of the destruction by rotting of a considerable portion of the fiber. Because of the expense of 35 separating the fiber the growing of flax for fiber has practically ceased for many years 40 in the United States and while flax is extensively grown it is grown only for its seed and the straw is practically a waste produce. While attempts have heretofore been made to get rid of the woody material by chemical 45 action the success of such attempts has not been such as to be commercially practical and the retting process is still the only process by which flax fiber is obtained commercially.

By the process of the present invention it 50 is now made possible without injury to the fiber, to quickly and effectively dissolve the resinous or gummy substances of the woody portion of the stalk to such an extent that it is rendered friable and is detached from 55 the fiber so that when the treated stalks or

straw is dried and subjected to the mechanical processes usually followed in the treatment of retted flax the fiber may be readily cleaned and made ready for spinning.

The result of the process of the present 60 invention is not only to reduce the time necessary to produce the clean fiber and thus materially reduce the cost of treatment of a given quantity of flax but to also secure a 65 much larger yield of fiber and to secure fiber of better quality than can be secured by the retting process.

In carrying out the process of the present invention the flax straw is taken as it comes from the field, either as dry straw or in a 70 green state, and is placed, preferably in bundles or sheaves, in a tank and there boiled in an alkaline degumming solution for about an hour and a half, at the end of which time the degumming solution is drawn off and 75 clean water introduced into the tank and agitated, preferably by introducing air under pressure at the bottom of the tank, so as to wash the treated straw to free it from the remains of the degumming solution. 80 After thus washing the treated straw the wash water is drawn off and an acid solution or sour bath solution is introduced into the tank and agitated so as to come in contact with all of the stalks or straws and neutralize any traces of alkali which might remain after the washing as well as to aid in completing the dissolving of the resinous or 85 gummy constituents of the woody portion of the stalks or straws. After the sour bath 90 solution has remained on the treated straw for about twenty minutes it is drawn off and the straw washed as before in clean water. The wash water having been drawn off a weak alkaline solution which may be termed 95 a "soap solution" is introduced into the tank and allowed to remain for a short time only preferably not over 10 or 15 minutes, the soap solution being preferably agitated while it remains on the straw. The soap 100 solution is then drawn off and the straw again washed. The chemical treatment of the straw is then complete and it only remains to separate the woody portion or shive of the stalk from the fiber from 105 which it has been loosened or detached by the action of the chemicals used. For this purpose the treated straw is dried by any convenient means and when dry the woody portion or shive is found to be so 110

friable that it is easily separated from the fiber by the ordinary methods employed for freeing retted flax from shives.

The fiber produced by the above described process is considerably greater in quantity than the amount produced by the retting process the chemicals used not attacking the fiber so that practically all of the fiber present in the stalk or straw is recovered as available for commercial use. The fiber produced by this process is much lighter in color than fiber produced by the retting process and is equally as strong if not stronger and is ready to be spun without bleaching though if desired it may be bleached by any usual bleaching process.

It will be noted that in the process as above described no preliminary deshiving of the flax straw is contemplated or desired and that the whole straw is carried through the several steps of the process without any separation of the shives or woody portion until the treatment is completed and the straw dried. By thus avoiding any mechanical treatment of the straw until it has been subjected to the complete chemical treatment any breaking of the fiber while it is still closely associated with the woody portion or shives is avoided.

30 The degumming solution is a solution in 20 gallons of water of five pounds caustic potash or caustic soda, 1 pound of borate of soda and  $1\frac{1}{2}$  pounds of sal-soda. The proportion of water may be varied to make 35 the solution stronger or weaker depending on the fibrous plant to be treated. The most satisfactory results are obtained by adding to this solution kerosene oil and linseed oil in the proportions of  $\frac{1}{2}$  gallon of 40 kerosene to 20 gallons of the solution and one quart of linseed oil. The kerosene appears to soften the resinous matters and to aid in dissolving them and the linseed oil appears to soften the fiber and render it less 45 likely to be injured in separating the shives from the dried straw.

The "sour bath" is a solution in 20 gallons of water of 6 ounces of sulfuric acid,  $\frac{1}{2}$  ounce of nitric acid and 4 ounces of acetic acid, though the proportion of water may be varied somewhat to make the solution stronger or weaker as may be found desirable.

The "soap solution" is a solution of potash and sal-soda in proportion of one part each of the potash and the sal-soda to ninety-eight parts of water.

The process has been above particularly described as applied to flax, but it is found 55 to be applicable with equally favorable results to jute, hemp, ramie and pita as well as to other fiber bearing plants the only

variation from the process as above described necessary in the treatment of fiber bearing plants other than flax being a variation in the strength of the degumming solution and the other solutions and a variation in the length of time required by the particular plant to be treated. 65

Having thus described the invention what I claim is:

1. The herein described process of degumming fibrous plants which consists in subjecting the stalks or straw to a boiling solution containing caustic potash, borate 75 of soda and sal soda and also containing hydrocarbon oil and vegetable oil.

2. The herein described process of degumming fibrous plants which consists in subjecting the stalks or straw to a boiling 80 solution containing caustic potash, borate of soda and sal soda and subsequently subjecting the stalks or straw to an acid bath containing an organic acid.

3. The herein described process of degumming fibrous plants which consists in subjecting the stalks or straw to a boiling solution containing caustic potash, borate of soda and sal soda and subsequently subjecting the stalks or straw successively to 90 an acid bath containing an organic acid and to an alkaline bath.

4. The herein described process of degumming fibrous plants which consists in subjecting the stalks or straw to a boiling 95 solution containing caustic potash, borate of soda and sal soda and also containing hydrocarbon oil and subsequently subjecting the stalks or straw to an acid solution containing an organic acid.

5. The herein described process of degumming fibrous plants which consists in subjecting the stalks or straw to a boiling solution containing caustic potash, borate of soda and sal soda and also containing 105 hydrocarbon oil and subsequently subjecting the stalks or straw successively to an acid bath containing an organic acid and to an alkaline bath.

6. The herein described degumming solution containing caustic potash, borate of soda and sal soda and also containing hydrocarbon oil and a vegetable oil.

7. The herein described degumming solution containing caustic potash, borate of 115 soda and sal soda in the proportions of 5 parts of caustic potash, 1 part of borate of soda and  $1\frac{1}{2}$  parts of sal soda and also containing hydrocarbon oil and vegetable oil.

This specification signed and witnessed. 120  
ROBERT R. ROBERTS.

In the presence of—

B. F. HAND,

D. E. BECKWITH.